

## UNITED STATES PATENT OFFICE

2,128,570

## FLOTATION MATERIAL

Merrill W. MacAfee, Berkeley, Calif., assignor to  
Great Western Electro-Chemical Company, a  
corporation of California

No Drawing. Application September 17, 1935,  
Serial No. 40,929

7 Claims. (Cl. 209—166)

This invention relates to a composition of matter useful in flotation. More particularly this invention is concerned with provision of a composition of matter enabling dixanthogens to be employed in flotation.

As is well known, dixanthogens are obtained from the oxidation of xanthates by oxidizing agents. Their use in flotation has heretofore been suggested and investigated. However, they have not gone into wide application. Gaudin in "Flotation," McGraw-Hill Book Company, 1932, at page 72, states that "unlike the alkali xanthates, dixanthogens are very little soluble in water. Their insolubility is one of the factors that has mitigated against their general use in sulphide flotation." This statement is quite true and very few mills in this country utilized dixanthogens on a commercial scale, prior to the present invention. The water insolubility of the dixanthogens has made it difficult to feed them properly as well as preventing their adequate incorporation in the pulp undergoing flotation. Dixanthogens have been added in ball mills to the ore being ground but this is only partly successful.

In accordance with this invention, I have been able to feed dixanthogens with accuracy and incorporate them directly in the pulp undergoing flotation. The result is that mills are accepting dixanthogens for commercial operation because they are able to achieve results not possible with the best flotation agents known heretofore, such as potassium ethyl xanthate, potassium secondary butyl xanthate and potassium amyloxanthate as well as the dithiophosphate compounds.

I have observed that flotation reagents such as dixanthogens tend to depress the froth during the flotation operation. This further complicates the operation and mitigates against the employment of the dixanthogens. I have found that both these undesirable effects of dixanthogen can be overcome by incorporating the dixanthogen in a suitable solvent therefor, preferably one which is not a frothing agent per se but which nevertheless neutralizes and offsets the depressing effect on the froth of the reagent. Such a solvent I have found in the alcohols such as methanol, isopropyl alcohol, secondary butyl alcohol, primary butyl alcohol, amyl alcohol, Pentasol (a mixture of amyl alcohols), and the various primary, secondary and tertiary amyl alcohols, and other organic solvents such as acetone. Any solvent can be used which is water miscible, of low vapor pressure and miscible with the dixanthogen.

The solvent employed is preferably anhydrous and anhydrous ethyl alcohol can be used although the ordinary commercial form includes such a percentage of water that only about a 5% concentration of the reagent can be secured. An 5 anhydrous solvent is desirable for water limits the quantity of dixanthogen which the solvent will carry. When the solvent carrying the dixanthogen is added to the water in the flotation circuit, the solvent, being water soluble, leaves 10 the dixanthogen behind but in a very well dispersed condition. In practice I usually make up a 50-50 mix by weight of the reagent and alcohol. This mixture is characterized by its 15 stability under ordinary conditions, a factor of 20 importance and one which usual solvents do not possess. The solvent also preferably has a low vapor pressure at ordinary temperatures for otherwise it will evaporate in the feeder to leave the dixanthogen remaining. It is also preferably 25 non-hygroscopic because if it is otherwise it will precipitate dixanthogen upon exposure to the atmosphere.

It is to be noted that the solvents employed are not frothing agents. I prefer not to incorporate the flotation reagents in frothing agents such as pine oil and the like because of the great power of the dixanthogens in flotation. Thus I have successfully floated minerals with the composition of the present invention using very 30 minute quantities while larger quantities of a frothing agent were necessary. By utilizing a solvent which is not a frother, the froth control and the flotation reagent control are simplified. The reagent of this invention can be readily 35 used in flotation after the manner of the Douglass Patent No. 1,943,758 and my prior Patent No. 2,061,201.

The use of the solvents of the present invention is to be further distinguished from this 40 prior art practice where in one flotation reagent would be incorporated a second agent, the second agent acting as a solvent for the first and having the additional capacity of also acting as a mineral collector. In this instance, the second 45 agent is used to neutralize the froth depressing effect of the first reagent and is in itself incapable of effecting an appreciable mineral recovery.

The invention is applicable to any dixanthogen whether aryl or alkyl and whether it is derived 50 from a primary, a secondary or a tertiary alcohol. It includes particularly the dixanthogens of such alcohols as ethyl, propyl, butyl and amyl alcohol, and their isomers as well as the secondary alcohols, iso-propyl, secondary butyl, 55

diethyl carbinol, methyl propyl carbinol, methyl isopropyl carbinol as well as tertiary alcohols of the same kind.

- 5 The preferred solvent is secondary butyl alcohol while the preferred dixanthogen is secondary butyl dixanthogen. These are made up in about equal parts by weight, the alcohol being anhydrous so it will carry this large quantity of dixanthogen.
- 10 10 Addition of the material of this invention, a dixanthogen in a diluted condition with a water soluble solvent therefor, has enabled results to be secured which are not obtainable with the same dixanthogens in their concentrated state.
- 15 15 This I attribute to activation of the dixanthogen, for, so far as the ore is concerned, the use of diluted dixanthogen gives recoveries not secured with a concentrated material. These results have been particularly evident on gold and silver 20 20 ores, particularly in the lead separation from the gold and silver ore at El Potosi mine in Mexico.

I claim:

1. As a composition of matter, a dixanthogen 25 dissolved in a substantially anhydrous water soluble aliphatic monohydric alcohol, said alcohol being water miscible and having a frothing power only sufficient substantially to offset any froth depressant power of said dixanthogen.

2. As a composition of matter, a dixanthogen dissolved in secondary butyl alcohol.

3. As a composition of matter, a dixanthogen dissolved in secondary amyl alcohol.

4. As a composition of matter, a secondary butyl dixanthogen dissolved in secondary butyl 5 alcohol.

5. As a composition of matter, a dixanthogen dissolved in a substantially anhydrous water soluble aliphatic monohydric alcohol, said alcohol being water miscible and having a frothing power only sufficient substantially to offset any froth depressant power of said dixanthogen, and being present in the mixture with said dixanthogen in about an equal weight. 10

6. In the process of concentrating ores and 15 minerals by flotation, the step which comprises subjecting the ore in the form of a pulp to a froth flotation operation in the presence of a dixanthogen diluted with a substantially anhydrous water miscible aliphatic monohydric alcohol as a solvent for the dixanthogen prior to incorporation of the dixanthogen in the pulp. 20

7. As a composition of matter, a dixanthogen dissolved in a substantially anhydrous secondary 25 aliphatic monohydric saturated unsubstituted alcohol.

MERRILL W. MACAFEE.